

April 16, 1940.

G. MALMGREN

2,197,133

## ELECTRICAL AMALGAMATOR

Filed June 28, 1937

2 Sheets-Sheet 1

Fig. 2.



Fig. 4.



Fig. 5.



Fig. 7.



INVENTOR,  
*GEORGE MALMGREN.*

BY

GEORGE MALMGREN.

ATTORNEYS.

April 16, 1940.

G. MALMGREN

2,197,133

ELECTRICAL AMALGAMATOR

Filed June 28, 1937

2 Sheets-Sheet 2.

Fig. 8.



INVENTOR,

GEORGE MALMGREN.

BY

*Lippincott & Metcalf*

ATTORNEYS.

## UNITED STATES PATENT OFFICE

2,197,133

## ELECTRICAL AMALGAMATOR

George Malmgren, Santa Cruz, Calif.

Application June 28, 1937, Serial No. 150,792

9 Claims. (Cl. 209—175)

My invention relates to a means and method for electrical amalgamation, and my invention is particularly desirable in the recovery of gold, silver, and platinum values from sands, gravels or classified ores.

Among the objects of my invention are: To provide an amalgamator having a continuous mercury flow; to provide an amalgamator utilizing the amalgamating plates as one pole of a galvanic battery; to provide an amalgamator utilizing electrical couples for cleaning mercury during amalgamation; to provide a means and method of electrical amalgamation; to provide a means and method of continuously removing values from an amalgamated plate; to provide an amalgamator utilizing intermittent electrical energization; and to provide an efficient and continuous means and method of segregating values from a metal bearing pulp.

My invention possesses numerous other objects and features of advantage, some of which, together with the foregoing, will be set forth in the following description of specific apparatus embodying and utilizing my novel method. It is therefore to be understood that my method is applicable to other apparatus, and that I do not limit myself, in any way, to the apparatus of the present application, as I may adopt various other apparatus embodiments, utilizing the method, within the scope of the appended claims.

In the drawings:

Figure 1 is a diagrammatic, longitudinal sectional view of a series of deck trays employing my invention.

Figure 2 is a cross-sectional view taken as indicated by line 2—2 in Figure 1.

Figure 3 is a cross-sectional view taken as indicated by line 3—3 in Figure 1.

Figure 4 is a cross-sectional view taken as indicated by line 4—4 in Figure 1 with the addition of a circuit diagram.

Figure 5 is a top view of a portion of a deck tray.

Figure 6 is a view partly in cross-section and partly in elevation and diagrammatic, to show one means of rocking the deck trays.

Figure 7 is a side view diagram showing how the deck trays are inclined.

Figure 8 is a flow sheet of one preferred setup of my invention.

Referring to the drawings for a more detailed description of my invention, a pulp carrying values of gold, silver, or platinum, or in fact any other metals that will amalgamate, is preferably

first screened wet to minus 16 mesh size, using a dilute solution of sodium or potassium sulphate, or a mixture of both, for the wash water, and I may also add the same solutions to the pulp until a suitable consistency is obtained to secure maximum recovery of the precious metals contained in the pulp. The ratio between solutions and solids for maximum recovery has to be established for each particular deposit by experimental runs. These solutions of sodium and potassium salts will hereafter be referred to as the electrolyte.

The pulp is then fed into a feed box 1, from whence it flows into deck trays 2, 3, and 4, placed on an angle and overlapped so that the pulp will run from one into the next. The deck trays 2, 3, and 4, are preferably made of copper and have an amalgamated mercury inner surface. Metallic mercury is continually fed to the top of the surface just before the pulp enters tray 2, through a mercury tube 5 from a mercury container 6, and sufficient mercury is continually fed so that there is, by gravity and by the action of the pulp on the surface of the mercury, a continuous flow of mercury over the amalgamated surface. In order to check the speed of the mercury flow and to add a riffling action to the amalgamator flow, I may wish to place a cross riffle 7 within one or more of the copper trays.

After the pulp has passed over the copper trays 2, 3, and 4, it passes into a main mercury trap tray 8. This tray differs from the prior trays in that it has a metal base plate 9, preferably iron, on which a copper plate 10 is fitted, the copper plate only being amalgamated, and at the lower end of the trap tray 8 there is a main mercury trap 11 extending across the tray. The amalgamated plate 10 extends into the mercury trap 11, and at the side of the trap, as shown in Figure 2, there is a mercury removal valve 12 through which the mercury may be allowed to pass continuously in accordance with the rate of arrival in the trap. This mercury will contain the greater portion of the values recovered, and is then treated for the removal of these values. The cleaned and condensed mercury may then be returned to mercury container 6.

If for any reason all of the mercury is not caught in the main mercury trap 11, it may be collected in an auxiliary mercury trap 14 which is identical with the mercury trap 11. A cross-section of the auxiliary mercury trap is shown in Figure 3, and the mercury collected therein may be periodically removed through mercury re-

moval tube 15. After the pulp has passed over the auxiliary mercury trap 14, it passes over the final apron 16 into settling tanks for separation of alkali salts from pulp tailings.

5 Immediately above all of the deck trays, including the mercury trap trays 11 and 14, I prefer to position zinc electrodes 17, all of them being connected in parallel. These electrodes are composed of cross bars 20 connected to upright sides 10 10 21, the cross bars being positioned above and parallel to the amalgamated surfaces. The zinc 15 plates are held in position by having the side walls 21 fastened to tray walls 24 by insulating blocks 25. I prefer to have the fastening adjustable.

15 A connection 26 is made to the trays, and a connection 27 is made to the zinc plates. A double throw switch 29 is provided so that the external circuit between connections 26 and 27, 20 and consequently the galvanic cell formed by the zinc plates and the trays may be shorted in one position of the switch. At the other position of the switch an exterior source of potential 30 may be applied in series with the 25 galvanic cell formed by the zinc plates and the trays.

I prefer, also, to set up the entire device in a sub-frame 31 mounted on hinged arms 32, the latter being also hinged to a base 34. A prime 30 mover 35 drives a crank 36 which is attached by a connecting arm 37 to one of the arms 32, the end of the arm 37 being mounted in a slot 39 in that arm so that a variable throw may be obtained by moving the end of the arm 37 along 35 the slot. The entire foundation 34 is mounted on graduated blocks 40 to obtain the proper inclination.

Having thus described the mechanical setup of my invention, I will now describe the method 40 of operation.

As before stated, the pulp is fed into the hopper 1 and passes along the inclined trays over the mercury surfaces. The pulp and electrolyte as referred to above is fed to the trays in sufficient amounts so that the pulp forms a layer 41, as shown in Figure 4, just below the zinc plate 17, but I prefer to have enough electrolyte in with the pulp so that the electrolyte layer 42 extends over the zinc bars 20. It is to be understood, however, that there will not always be a definite line of demarcation between pulp and electrolyte such as has been shown in Figure 4, only the heavier portions of the pulp being below the zinc plates. In any event, I wish to have the 55 zinc plates well covered to obtain proper galvanic action.

After the continuous stream of mercury has been started and the pulp flows through the device, the chemistry of the amalgamation 60 comprises the use of a galvanic cell in which the negative electrodes are the zinc plates 17. In this respect I do not wish to be limited to the use of zinc, as any metal suitable because of its position in the electromotive force series may be utilized. The positive electrode is the mercury 65 surface of the amalgamated plates and the electrolyte is the dilute solution of the sodium or potassium salts that is added to the pulp. Since in the E. M. F. series zinc is .770 volt negative 70 relative to hydrogen, and mercury is .748 volt positive to hydrogen, there will be a total E. M. F. of 1.518 volts between the two electrodes when no current is passing through the cell. If the circuit is completed through the external switch 75 29, a current flows from the zinc plate to the

mercury on the trays. This galvanic current dissociates the sodium and potassium salts, frees the alkali metal from solution, and the alkali metal is then deposited on the surface of the mercury and immediately amalgamates therewith. The water present in the electrolyte acts on the freshly deposited alkali metal, producing a hydroxide. This reaction keeps the surface of the mercury clean and active, as the cell is shorted during recovery except for the intermittent use of external voltage hereafter described.

When a particle of gold, for example, is brought into contact with the mercury by concentration from the pulp, the galvanic action at the point 15 of contact of the mercury with the gold is in intensified due to the fact that a new galvanic couple is formed, with the zinc acting as a negative and the gold acting as a positive electrode. Since gold is 1.079 volts positive relative 20 to hydrogen, the galvanic action is intensified and the subsequent electrolytic action accelerates the rate of amalgamation of the gold.

With regard to the particular type of electrolyte used in practice, I have found that by 25 using sodium sulphate alone I have obtained good recovery of gold and fair recovery of silver. The use of small percentages of potassium sulphate with the sodium sulphate has increased the recovery in such cases where the pulp contained 30 minerals that discolored the bright mercury surface. Too much potassium salt renders recovery more difficult in that so much hydrogen is generated that the gold does not come in contact with the amalgamated surface, and I have found 35 that one good electrolyte ratio is five per cent  $K_2SO_4$  and ninety-five per cent  $NaK_2SO_4$  solutions. I have also found that it is advisable to adjust the relative position of the zinc plates with relation to the deck trays in order that the 40 internal resistance may be adjusted and the pulp space changed.

While I have shown a double throw switch 45 which may be utilized to short circuit the galvanic cell as above described or to additionally energize the cell, I prefer at all times to utilize the external current through the cell intermittently, inasmuch as I have found that intermittent action gives me a far higher recovery than can be possibly obtained by constant action. Intermittent 50 use, however, gives consistent and efficient removal, and often the period can be determined by watching the mercury surfaces to determine the brilliance thereof. The current is used only when the mercury surface dulls. In practice, 55 short energization periods at intervals of fifteen minutes has been found sufficient with some ores.

The external current source which may be utilized by means of the double throw switch 29, is only used when it is necessary to clean 60 the deck plates due to heavy contamination by certain minerals occurring in the deposit, or when it is desired to amalgamate platinum or certain silver compounds occurring in nature. Even when the external source is utilized, however, the current is only used intermittently. For example, in the full or partial reduction of 65 certain sulphides, reddish brown spots are left on the mercury surface. These spots are easily removed by momentary use of the external 70 E. M. F.

With regard to platinum, it has been found that platinum does not amalgamate readily unless an external E. M. F. is used, and not at all if the same is used continuously. By far the 75

best results are obtained by intermittent use, the period being different, depending upon the other minerals to be recovered and the character of the deposit. It has also been found that the amalgamation is not particularly rapid if only an external E. M. F. is used, that is, when the amalgamator itself is not a galvanic cell.

From the tests which I have made comparing weighed samples of ore treated in various ways including the process described above, I am inclined to believe that a high recovery is obtained because the galvanic action increases the settling of the fine slimes and cleans all surfaces and value particles. I have also found that the sulphides in the tailings were clean and bright. Other tests have shown that gold which is dirty or greasy is rapidly and efficiently amalgamated, probably due to the action of the caustic alkalies developed during the passage over the deck trays. Tests conducted with naturally coated gold showed that the humic acid of which the coating is mostly made up, in some manner combines with the alkali salts or with the metallic alkali metals deposited by the galvanic action, and that the mercury spreads over the gold and amalgamates it, leaving nothing but a few grains of silica and iron oxide on the surface of the mercury.

I have, therefore, by the use of the process above described and the preferred form of apparatus, been able to make high recoveries, particularly of the finer values in pulp, and my process has the advantage that it is continuous, with a continuous removal of the values without the necessity of shutting down the flow. In that regard, the continuity of my preferred setup is shown in Figure 8, where the pulp, alkali salts, and mercury are fed to the amalgam plates and the amalgam is continuously removed, treated to recover the precious metals, and the mercury returned to the input end. In like manner the discharge from the amalgam plates may be run in a settling tank, the salts removed and passed back to the input end of the device, and the tailings further treated chemically if desired.

While I have described my preferred form of apparatus as utilizing copper amalgam plates, it is within the knowledge of those skilled in the art to use equivalent amalgam plates, as for example, silver plates, and it is also within the knowledge of those skilled in the art to rearrange, extend, or change the tray setup within the scope of the appended claims.

I claim:

1. The method of recovering metal values from a wet pulp by amalgamation with mercury which comprises mixing an alkaline electrolyte with said pulp, passing the resultant pulp over a mercury surface, immersing a material electro-negative to the amalgamated surface in said pulp, and directly shorting said material to said surface.

2. The method of recovering metal values from a wet pulp by amalgamation with mercury which comprises mixing an alkali metal sulphate electrolyte with said pulp, passing the resultant pulp over a mercury surface, immersing a material electro-negative to the amalgamated surface in said pulp, and directly shorting said material to said surface.

3. The method of recovering metal values from a wet pulp by amalgamation with mercury which comprises mixing an alkali metal sulphate electrolyte with said pulp, passing the resultant pulp

over a mercury surface, immersing a material electro-negative to the amalgamated surface in said pulp, and directly shorting said material to said surface.

4. The method of recovering metal values from a wet pulp by amalgamation with mercury which comprises mixing an alkali metal salt electrolyte with said pulp, passing the resultant pulp over a mercury surface, utilizing said mercury surface as the positive pole of a galvanic cell in said electrolytic pulp, and shorting said cell.

5. The method of electrically cleaning a mercury surface covered by a value bearing pulp which comprises adding an alkali metal salt solution to said pulp, passing the wet pulp over said surface, immersing a material electro-negative to the amalgamated surface in said pulp, directly shorting said material to said surface, and cleaning said surface by intermittently passing additional current through said pulp to said surface.

6. An amalgamator comprising an inclined tray, a mercury amalgamated surface on the bottom of said tray, means for introducing a wet value bearing pulp including an electrolyte at the high end of said tray, means for simultaneously introducing metallic mercury at the high end of said tray, means for separating the pulp and mercury at the low end of said tray, an electronegative electrode positioned over a substantial area of said mercury surface, insulated therefrom and immersed in said pulp, and external means for shorting said electrode and said surface.

7. An amalgamator comprising an inclined tray, a mercury amalgamated surface on the bottom of said tray, means for introducing a wet value bearing pulp including an electrolyte at the high end of said tray, means for simultaneously introducing metallic mercury at the high end of said tray, means for separating the pulp and mercury at the low end of said tray, an electronegative electrode positioned over a substantial area of said mercury surface, insulated therefrom and immersed in said pulp, external means for shorting said electrode to said surface, means for alternatively and intermittently placing an exterior source of potential in series with the galvanic cell formed by said electrode and said surface in said pulp.

8. The method of recovering metal values from a wet pulp by amalgamation, comprising adding to the pulp an electrolyte composed of approximately ninety-five per cent of sodium sulphate and approximately five per cent of potassium sulphate, passing said pulp between and in contact with a pair of interconnected electrodes occupying different positions in the electromotive series to create galvanic action through the reaction of said electrolyte and said electrodes, one of said electrodes containing mercury, and causing the formation of temporary localized galvanic couples by the deposition of particles of such values on the surface of said mercury containing electrode.

9. The method of recovering metal values from a wet pulp by amalgamation, comprising adding an electrolyte to such pulp, passing said pulp between and in contact with a pair of electrodes, one of which includes mercury, exposing such pulp to a continuous flow of current of a relatively low magnitude between said electrodes and intermittently increasing the magnitude of such current.

GEORGE MALMGREN.